

1

2,773,031

## DRILLING MUDS

Rodolfo J. Tailleur, San Tome, Venezuela, assignor to Gulf Oil Corporation, Pittsburgh, Pa., a corporation of Pennsylvania

No Drawing. Application October 28, 1954,  
Serial No. 465,418

21 Claims. (Cl. 252—8.5)

This invention relates to improvements in drilling mud compositions of the type used in well drilling, and more particularly it pertains to oil-in-water emulsion drilling muds having improved lubricating properties.

A substantial portion of the total time consumed during well drilling operations is taken up in the replacement of drill bits. Inasmuch as changing a bit necessitates pulling the entire string of drill stem, substituting a new bit, and rerunning the entire string of drill stem back into the borehole, it is evident that the time consumed in making bit changes increases roughly in proportion to the depth being drilled. As wells are being drilled to ever increasing depths, the economic losses attendant upon the increasing amount of time lost in making bit changes cannot be ignored. In addition to the loss of time involved in making bit changes, the necessity for making frequent bit changes, particularly when drilling at substantial depths, may create hazards, such as increasing the likelihood of cave-ins, which may arise as a result of stopping the circulation of the drilling mud during the change of bits.

Obviously, the necessity for making a bit change is dictated by the exhaustion of the useful life of the bit. Although much has been done toward improving drill bits and drilling techniques in order to prolong useful life, in the present state of rotary bit development, the most frequent limiting factor of bit life is failure of the bearings, rather than the cutting teeth.

Thus, perhaps the most important factor tending to shorten the useful life of a drill bit is the lack of adequate lubrication of the bearings. In the past, efforts have been made to afford lubrication for the bearings by incorporating self-contained lubricating units in the bits. That such efforts have not been entirely successful is borne out by the fact that conventional bits currently in use are not provided with such self-lubricating units. Consequently, conventional bits receive only such lubrication as may be obtained from the drilling mud being circulated therethrough. Since the bearings of the bit are subjected to high loads, the value of conventional drilling muds as bit lubricants leaves much to be desired.

Although lubricating properties have commonly been attributed to conventional oil-in-water emulsion drilling muds, as far as I am aware, it has not been satisfactorily demonstrated that such muds actually behave as lubricants for the bearings of drill bits under actual field conditions which impose high specific loads on the bearings of the bit. I have investigated some commonly used oil-in-water emulsion drilling muds to which lubricating properties have been attributed, and on the basis of field tests and tests made with the Timken wear and lubricant tester, I have found that the lubricating properties of such muds are of no significance with respect to the specific loads on the bearings under the conditions to which a drill bit is subjected in the field. In other words, under such conditions, such muds have practically no lubricating value for the bearings of drill bits.

I have now discovered that oil-in-water emulsion drill-

2

ing muds can be made to possess effective lubricating properties and thus prolong the life of drill bits while retaining the normally desirable properties of such muds. In accordance with my invention, I provide a drilling mud which is an emulsion of oil-in-water containing clay solids, and an asphalt in the oil phase, said asphalt having chemically combined sulfur and being present in an amount sufficient to provide at least about one percent of sulfur by weight of the oil phase. Such drilling muds possess excellent lubricating qualities and prolong the life of the bearings of drill bits, thereby reducing the frequency of bit changes and decreasing the time diverted from actual drilling operations.

The asphalts utilized in the muds of my invention include such materials as natural asphalts, petroleum asphalts, reduced crudes, blown asphalts, the solid petroleum residues or pitches obtained in the vacuum reduction of crude oils and such asphaltites as manjak or glance pitch and grahamite, provided that the foregoing materials contain such an amount of sulfur that upon incorporation into the oil phase of the drilling muds they provide at least about one percent of sulfur by weight of the oil phase.

It will be understood by those skilled in the art that the sulfur content of various asphalts will vary, depending on their source and/or the specific methods by which they have been prepared. For example, crude asphaltic petroleum oils high in sulfur may yield asphalts of a relatively high sulfur content if the sulfur tends to concentrate in the residual fractions during distillation. Similarly, the depth of reduction of an asphaltic crude oil can determine the sulfur content of the asphalt residues obtained. Among the natural asphalts, the sulfur content appears to depend primarily on the source of the asphalt, although in the case of the asphaltites the type of asphaltite is important, manjak and grahamite containing sufficient amounts of sulfur whereas gilsonite does not. In general, in order to provide the desired sulfur content in the oil phase, and having regard for the asphalt concentration in the oil phase as will be elaborated below, the asphaltic materials employed in the oil phase must contain at least about 1.5 percent of sulfur by weight. As is known in the art, the sulfur in such asphaltic materials is chemically combined in the form of sulfur-hydrocarbon complexes of high molecular weight.

The asphalts themselves are well-known materials, the properties and preparation of which have been detailed in the art. They range from highly viscous liquids to semi-solid to essentially solid materials. Since the asphalts in the muds of my invention are part of the oil phase, it is desirable that they dissolve or disperse readily to become uniformly blended in the oil employed in the oil phase. The preferred asphaltic materials are therefore those of a relatively high sulfur content, possessing the property of ready solubility or dispersibility in the distillate petroleum fractions commonly employed in the oil phase of oil-in-water emulsion drilling muds. For example, one preferred asphaltic material is a reduced Kuwait crude from the Burgan field, having a flash point of about 650° F. or somewhat higher and a sulfur content of about 5.2 percent. This material is readily dispersed in a gas oil of the diesel fuel type without any difficulty, for example, in proportions of reduced crude to diesel fuel ranging from 1:1 to 3:1 by volume. Similarly, there exist other asphalt-containing petroleum residues of a relatively high sulfur content, for example, residues obtained from Eastern and Western Venezuelan crudes, Iranian crudes and West Texas crudes, which can be cut back or thinned with a petroleum distillate fraction, such as a light or heavy catalytically cracked cycle oil in the gas oil boiling range, and these constitute preferred materials.

It is also possible to obtain the desired sulfur- and asphalt-containing oil phase by employing as the oil phase in the muds of my invention a residual fuel oil of the type of No. 6 fuel oil, such oils being available with sulfur contents of from about 2 to 3.5 percent. Similarly, topped or reduced crudes containing sufficient sulfur can be cut back or thinned with suitable petroleum solvents to form the entire oil phase. In some instances, depending upon the nature of the crude oil, it is possible to employ the entire residue from a topping operation as the oil phase, such topping residues containing sufficient asphaltic material of the desired sulfur content and sufficient oil to make up the remainder of the oil phase.

In the event more difficultly soluble asphaltic materials are employed, it is desirable to employ in the oil phase oils of higher solvency such as highly aromatic petroleum distillates or the liquid extracts obtained in the solvent refining of lubricating oils. Additionally or alternatively, an auxiliary solvent or blending agent, for example, liquid chlorinated diphenyl or the above-mentioned liquid solvent extracts can be employed to obtain the desired uniform blend of the asphalt in the oil phase. Incorporation of the asphalts in the oil phase can also be facilitated by initially melting or finely dividing the material prior to adding the oil, and/or heating the oil-asphalt mixture to about 180° F.

The amount of sulfur-containing asphalt employed in the oil phase to provide at least about one percent of sulfur by weight of the oil phase will vary with the sulfur content of the particular asphaltic material employed. For example, with an asphaltic material such as a manjak containing about 10 percent by weight of sulfur, at least 10 percent of the manjak must be employed to obtain a sulfur content of at least one percent of the oil phase. With asphaltic materials containing less sulfur, larger amounts of asphalt must be employed. As a practical maximum, it is undesirable to employ more than about 75 percent by weight of asphalt in the oil phase because there are then obtained unstable emulsions which tend to foam excessively. Furthermore, the viscosity of the oil phase containing such large amounts of asphalt is so high as to approach the solid state, causing difficulties in handling at the well site. Accordingly, the asphalt should contain not less than about 1.5 percent of sulfur to provide the necessary sulfur content in the oil phase without encountering the above-mentioned difficulties.

Since the oil phase of my oil-in-water emulsion drilling muds contains substantial amounts of asphaltic materials, as has been shown hereinabove, the oil employed in the oil phase is a non-residual or distillate oil, such as gas oils, kerosenes, diesel fuel oils, distillate lubricating oils, the liquid extract fractions obtained in the solvent refining of lubricating oils, or mixtures of such oils. It has already been pointed out in connection with the description of the sulfur-containing asphalts that certain of the latter materials can be obtained in solution in petroleum distillates. In such instances, the further addition of a distillate oil to such asphalt-containing materials is ordinarily unnecessary, particular reference being made to the asphalt cutbacks, residual fuel oils and the topped crudes containing sufficient distillate fractions, as already described, which constitute the entire oil phase. The total oil phase of the drilling muds of the invention ranges from about 2 to 40 percent by volume of the entire drilling mud, preferably from about 5 to 25 percent. The emulsifying agent, presently to be described, is also considered to be part of the oil phase for the purpose of determining the amount of total oil phase in the mud.

Since the drilling muds of my invention are oil-in-water emulsion drilling muds, an emulsifying agent will normally be added during preparation of the muds to facilitate emulsification or dispersion of the oil phase in the water phase and to stabilize the emulsion obtained.

Numerous emulsifying agents for preparing oil-in-water emulsions are known in the art and any of such conventional emulsifying agents can be employed for the above purposes.

However, in the use under drilling conditions of oil-in-water emulsion drilling muds, it is desirable that the mud filtrate have a low surface tension, say on the order of 40 dynes per centimeter or below. Since emulsifying agents are surface-active compounds, they will also act to reduce the surface tension of the filtrate, although not all emulsifying agents are of equal effect for this purpose. In a preferred embodiment of my invention, my drilling muds therefore contain an emulsifying agent which not only serves to assist in the emulsification of the oil and to stabilize the emulsions formed, but substantially to reduce the surface tension of the filtrate as well. I have found that emulsifying agents which are particularly suitable for the latter purpose include preferably oil-soluble alkylaryl sulfonic acids, e. g., "wax" benzene sulfonic acids and mahogany acids, and metal salts thereof, e. g., the alkali metal, ammonium and alkaline earth metal, including calcium and magnesium, salts. Other suitable emulsifying agents include the sodium soaps of tall oil and the fatty acid esters of the anhydroalkitols, for example, sorbitan, mono-, di-, or tri-oleate, sorbitan mono-stearate, etc. Of the above emulsifying agents, I prefer to employ the sodium salt of mahogany acids, because not only is it more effective in achieving the desired reduction in surface tension of the filtrate, but it can be used in smaller amounts for this purpose than other emulsifying agents. Substantial economies can therefore be achieved.

In general, satisfactory results with respect to reducing the surface tension of the filtrate and stabilizing the emulsion can be obtained by the use of from about 1 to 4 pounds of emulsifying agent per barrel of the entire drilling mud composition, sufficient to reduce the surface tension of the filtrate substantially below that of water and preferably to about 40 dynes per centimeter or less. However, when using the preferred emulsifying agent, namely, the sodium salt of mahogany acids, it is highly advantageous to employ not more than about 2 pounds per barrel in order to avoid excessive oil loss in the filtrate, as fully set forth in my copending application, Serial No. 350,460, filed April 22, 1953, now U. S. Patent No. 2,713,032.

Any clay can be utilized in the drilling muds of this invention which is commonly employed for this purpose in the art. Such clays, which form dispersions or gels with water, can be native products, such as may be available at the well site, or a relatively pure clay, such as bentonite, or base-exchanged clays, such as lime-treated clays, etc. In general, when using clays such as bentonite, the clay is employed in an amount of from about 2 to 8 percent by weight of the entire composition, more or less, depending upon the yield (barrels of mud of 15 centipoise viscosity per ton of clay) of the clay. When native clays are employed, larger amounts, say as high as 40 percent by weight of the mud composition, can be used because they yield less barrels of mud per ton of clay.

It is characteristic of the drilling muds of this invention that they are sensitive to the presence of alkali metal hydroxides. By this I mean that the addition of substantial quantities of alkali metal hydroxide to these muds results in a loss of the lubricating properties otherwise obtained through the use of the sulfur-containing asphaltic material in the oil phase.

Similarly, a drilling mud which has already been treated with substantial amounts of alkali metal hydroxide does not respond beneficially to later treatment with the sulfur-containing asphalt. In other words, notwithstanding the fact that oil-in-water emulsion drilling muds contain a sulfur-containing asphalt, such muds will not have enhanced lubricating properties in the presence of alkali metal hydroxide. This phenomenon is unexpected and

cannot be satisfactorily explained at present, particularly since the lubricating properties of the muds of this invention are not detrimentally affected by admixture with such materials as calcium hydroxide or sodium chloride.

The sensitivity of the drilling muds to alkali metal hydroxide imposes certain precautions in the use of clay deflocculants to reduce the viscosity and fluid loss of the muds. For example, one of the most widely used clay deflocculants is quebracho which is generally employed with caustic soda. If the drilling muds of this invention are treated in the usual manner with the conventional quebracho-caustic soda mixture, there results a loss of the enhanced lubricating properties, although the otherwise normal properties of the muds are retained. It is to be noted, however, that the muds of the invention will tolerate a limited amount of caustic soda without losing their load-carrying capacities. The limits of such tolerance are difficult to specify exactly since they will vary with the nature and amount of the clay in the drilling mud. For example, with a drilling mud made in accordance with this invention, containing pure bentonite as the clay in an amount of 6 percent by weight of the entire mud and having a relatively high tolerance to alkali metal hydroxides, I have found that the use of 0.5 pound of caustic soda per barrel of drilling mud, although reducing the load-carrying capacity considerably, does not render the mud worthless from a lubricating standpoint. However, when the caustic soda is increased to 1.0 pound per barrel of the mud, the lubricating properties of the mud are substantially eliminated. With other clays, the caustic soda tolerance is substantially less.

From the foregoing, it will be apparent to those skilled in the art that no substantial amount of caustic soda should be added to the muds of this invention; in no event should such amount be sufficient to destroy the enhanced lubricating properties of the muds. Since in normal field practice, the amounts of caustic soda usually employed, particularly in connection with quebracho treatment, are in substantial excess of the amounts deleteriously affecting the lubricating properties of the muds of the invention, when it becomes desirable to use an alkaline treating agent with or without a clay deflocculant, it is preferred to employ such alkaline materials as ammonia, amines, such as mono-, di- and triethanolamine, etc. which do not have any deleterious effect on the lubricating properties of the muds. In treating the muds of my invention with quebracho, it is possible to use this material alone, that is, without the joint use of caustic soda, although in such case more of the quebracho will usually be required to obtain the desired deflocculating effect.

In the actual practice of my invention, it is permissible to conduct the entire drilling operation with the drilling muds above described. However, initial drilling operations can be started with a conventional straight water-base mud because the soft formations and the absence of high specific loads on the drill bit at the shallower depths do not require greater lubricating properties than can be obtained with a water-base mud. Thereafter, as dictated by the requirements of drilling and the formations encountered, the water-base mud is converted to the mud of my invention. This conversion can readily be accomplished during circulation of the water-base drilling mud in the well by adding to the mud in the mud pit a sulfur-containing asphalt and an oil, either separately or in admixture in the form of a cut-back, and an emulsifying agent. These materials are added in an amount dependent upon the total amount of the drilling mud already in the system and preferably at a rate dependent upon the rate of drilling mud circulation, so as to effect a substantially uniform dispersion of the oily materials as an oil phase throughout the drilling mud system. Conventional methods can be employed for whatever mechanical agitation is necessary to achieve proper mixing. It is highly desirable to add the

emulsifying agent to the water-base drilling mud in admixture with the oil, but if added separately, it is advisable that it be added after the oil has been added or simultaneously with the addition of the oil. If the emulsifying agent is added prior to addition of the oil phase, there is a tendency for the mud to foam excessively and this entails the risk of a blowout.

In the practice of my invention, it is also possible to convert an existing conventional oil-in-water emulsion drilling mud to a drilling mud in accordance with my invention. This is also accomplished during circulation of the drilling mud in the well by adding thereto, with agitation with the drilling mud in the usual mud pit, a sulfur-containing asphalt or a concentrate thereof in oil. The concentrate can also contain an emulsifying agent. The total amount of sulfur-containing asphalt or the oil concentrate thereof and the concentration of the components therein are such that the concentration of the components of the resulting drilling mud composition being prepared, taking into account the composition of the conventional oil-in-water emulsion drilling mud being converted, will result in an oil-in-water emulsion drilling mud having the composition of the muds of my invention, as set forth in detail above.

It will be understood that the drilling muds of my invention which have become depleted in one or more components during use can be treated with the depleted components or oil concentrates thereof to restore the desired concentration of such components.

As an example of the preparation and use of one of the preferred embodiments of my invention in drilling a well, about the first two thousand feet of hole are drilled using as the drilling mud the mud formed from water and the natural clays incorporated therein from the formations during the drilling. In case such formations are deficient in natural clays, it is permissible to add a small quantity of bentonite to the drilling mud to increase the viscosity and thixotropic and wall building properties thereof. Up to this point, the procedure is identical with normal drilling operations where straight water-base drilling muds are employed. At this stage, the water-base drilling mud in the system totals about 500 barrels (barrel throughout the specification and claims is 42 standard U. S. gallons). It having been determined that conversion to an oil-in-water emulsion drilling mud is now desirable, an oil phase is prepared as follows. Into a suitable mixing vessel, there are placed 11.5 barrels of a diesel fuel oil, 34.5 barrels of a reduced Kuwait crude from the Burgan field, having an API gravity of 5.9, a flash point of 665° F. and a sulfur content of about 5.2 percent, and 4 barrels of an oil concentrate of the sodium salts of mahogany acids (the concentrate being available commercially as Petronate HL, containing 60 percent by weight of the salts dissolved in a lubricating oil). The mixture is stirred until all of the components are uniformly blended. The oily composition thus prepared, which is to constitute the oil phase of the drilling mud, amounts to about 50 barrels and is a moderately viscous, black liquid that can be pumped readily at ordinary temperatures and emulsifies readily in the mud to form an oil-in-water emulsion. The oily composition is then added to the straight water-base drilling mud by circulating the mud through the well while pouring the oily composition into the mud ditch through which drilling mud returns to the mud pits from the well and agitating the pits with mud guns. Drilling need not be discontinued during the change from a water-base mud to the oil-in-water emulsion mud of my invention. After all of the oily composition has been added to the pre-existing drilling mud and after the mixture has been circulated through the well about two or three times, the entire drilling mud in the system is a uniform oil-in-water emulsion mud of my invention. Continued drilling with the new mud results in the benefits and advantages heretofore described.

In the following illustrative examples, there are set forth certain specific embodiments of the drilling mud compositions of the invention. It will be understood that these specific embodiments are given by way of illustration only and are not intended to limit the invention. It will be noted that, in determining the improvement in lubricating properties of the drilling muds, I have employed the well-known Timken wear and lubricant tester. This machine is employed in the lubricating oil art to determine the load-carrying capacity of lubricants. It was obviously impractical to test the lubricating properties of all the drilling muds set forth in each of the specific examples in an actual well drilling operation, but I have found that the load-carrying capacities of drilling muds, as determined by the Timken machine, are a measure of the prolongation of bit life and other advantages obtained through the use of my drilling muds in actual drilling operations in the field. Since the load-carrying capacities of drilling muds as obtained by the Timken machine correlate well with actual field tests, it is thus possible to test the efficacy of drilling muds in the laboratory to determine their suitability for use in the field.

It is characteristic of the drilling muds of this invention that they have load-carrying capacities, as measured by the Timken machine, of not less than 30 pounds, as compared to load-carrying capacities of 15 pounds and below for conventional oil-in-water emulsion drilling muds which have substantially no lubricating properties.

There are set forth in the following table illustrative examples of drilling muds made in accordance with the invention. The table also includes for purposes of comparison a mud (Example 18) which represents the conventional oil-in-water emulsion muds of the prior art. All of the muds of the examples were prepared by the following general procedure. The oil, the asphaltic material and emulsifying agent were mixed, and the mixture was heated to 180° F. and stirred for 15 minutes to obtain a uniform blend of the various constituents. The oily mixture was then added to a suspension of 6 percent by weight of bentonite in water, and the entire mixture

100 grams after 5 seconds. The manjak had a sulfur content of 9.1 percent by weight. The reduced Kuwait crude had an API gravity of 5.9, a flash point of 665° F. and a sulfur content of about 5.2 percent.

5 Under the heading "Oil" in the table, the "Naphthenic Extract No. 1" was the oily material obtained as the extract fraction in the solvent extraction of a 400 Texas lubricating distillate with furfural. The extract had an API gravity of 14.5° and a viscosity of 1170 S.U.S. at 100° F. The "Diesel Fuel Oil" employed had a gravity of about 35° API, a flash point of about 178° F. and a boiling range of about 440° to 625° F.

Under the heading "Emulsifying Agent," the "Petronate" employed was an oil concentrate containing about

15 60 percent by weight of the sodium salts of mahogany acids, said sodium salts having an average molecular weight of from about 445 to 460. The "Calcium Petronate" was an oil concentrate containing 41 percent by weight of the calcium salts of mahogany acids having a molecular weight of 888. The "Magnesium Petronate" was an oil concentrate containing 47 percent by weight of the magnesium salts of mahogany acids having a molecular weight of 854. The "mahogany acids" employed were a 46 percent by weight concentrate in a lubricating

20 oil fraction of the preferentially oil-soluble petroleum sulfonic acids obtained as a by-product in the refining of lubricating oil fractions with oleum.

25 In Example 17, instead of bentonite, the clay employed was a calcium base-exchanged bentonite in a concentra-

30 30 of 6 percent by weight of its suspension in water. In preparing the calcium base-exchanged bentonite, a 2 percent by weight suspension of bentonite in water was treated with lime in the proportion of 3 pounds per barrel, well agitated and aged overnight. Thereafter, an

35 35 additional amount of dry bentonite was added, sufficient to give a total bentonite concentration in the suspension of 6 percent by weight. With the addition of the dry bentonite, there occurred a slight increase in viscosity of the mud. The mud was thinned by the addition of calcium lignosulfonate in the proportion of  $\frac{1}{2}$  pound per barrel.

| Example | Sulfur-Containing Asphalt  |                             |                                       | Oil                      |                                                  | Emulsifying Agent        |                 | Timken Load-Carrying Capacity (Pounds) |
|---------|----------------------------|-----------------------------|---------------------------------------|--------------------------|--------------------------------------------------|--------------------------|-----------------|----------------------------------------|
|         | Type                       | Percent by Wt. of Oil Phase | Percent by Wt. of Sulfur in Oil Phase | Type                     | Total Oil Phase, Percent by Vol. of Drilling Mud | Type                     | Lb./Bbl. of Mud |                                        |
| 1.      | Granular Petroleum Asphalt | 30                          | 1.0                                   | Naphthenic Extract No. 1 | 10                                               | Petronate                | 4               | 35                                     |
| 2.      | do                         | 50                          | 1.7                                   | do                       | 10                                               | do                       | 4               | 50                                     |
| 3.      | Manjak                     | 20                          | 1.8                                   | do                       | 10                                               | do                       | 3               | 55                                     |
| 4.      | Kuwait Reduced Crude       | 73                          | 3.8                                   | Diesel Fuel Oil          | 10                                               | do                       | 1               | 75                                     |
| 5.      | do                         | 71                          | 3.8                                   | do                       | 10                                               | do                       | 2               | 80                                     |
| 6.      | do                         | 68                          | 3.5                                   | do                       | 10                                               | do                       | 3               | 85                                     |
| 7.      | do                         | 68                          | 3.5                                   | do                       | 10                                               | do                       | 3               | 15*                                    |
| 8.      | do                         | 61                          | 3.2                                   | do                       | 10                                               | do                       | 3               | 90                                     |
| 9.      | do                         | 46                          | 2.4                                   | do                       | 10                                               | do                       | 3               | 60                                     |
| 10.     | do                         | 0.1                         | 0.5                                   | do                       | 10                                               | do                       | 3               | 10                                     |
| 11.     | do                         | 71                          | 3.8                                   | do                       | 10                                               | Sorbitan Monooleate      | 2               | >100                                   |
| 12.     | do                         | 71                          | 3.8                                   | do                       | 10                                               | Sorbitan Trifoleate      | 2               | 90                                     |
| 13.     | do                         | 68                          | 3.5                                   | do                       | 10                                               | Sodium Soaps of Tall Oil | 3               | >100                                   |
| 14.     | do                         | 66                          | 3.4                                   | do                       | 10                                               | Calcium Petronate        | 4               | 85                                     |
| 15.     | do                         | 73                          | 3.8                                   | do                       | 10                                               | Magnesium Petronate      | 1               | >100                                   |
| 16.     | do                         | 68                          | 3.5                                   | do                       | 10                                               | Mahogany Acids           | 3               | >100                                   |
| 17.     | do                         | 68                          | 3.5                                   | do                       | 10                                               | do                       | 3               | >100                                   |
| 18.     | do                         | 0                           | 0                                     | do                       | 10                                               | Petronate                | 3               | <5                                     |

was heated in an open vessel at 140° F. with sufficient stirring to insure complete emulsification. Prior to testing in the Timken machine, the oil-in-water emulsion muds thus prepared were placed in a sealed container and aged overnight.

Under the "Asphalt" column in the table, there are shown granular petroleum asphalt, manjak and Kuwait reduced crude. The granular petroleum asphalt employed had a sulfur content of about 3.5 percent, a melting point of 325° F. and penetrations of 0 at 77° F. and 2 to 3 at 115° F., both penetrations being measured under loads of

65 It will be noted from the above table that conventional oil-in-water emulsion drilling muds had substantially no lubricating properties. This is shown in Example 18, wherein the load-carrying capacity of a drilling mud containing 10 percent by volume of diesel fuel oil was less than 5 pounds. A mud of this type is substantially identical with oil-in-water emulsion muds commonly employed in the field. The addition of a sulfur-containing asphaltic material, in accordance with the invention, resulted in substantial increases in load-carrying capacity, ranging from the 35 pound figure shown in Example 1

to more than 100 pounds shown in the other examples.

Examples 6 and 7, taken together, show the effect of alkali metal hydroxides on the drilling muds of the invention. The asterisk adjacent the value of load-carrying capacity shown in Example 7 indicates that this mud has been treated with alkali metal hydroxide. Example 6 is a mud of the invention without having been treated with caustic soda and has a load-carrying capacity of 85 pounds. As shown in Example 7, when the mud of Example 6 was treated with 1 pound per barrel each of caustic soda and quebracho, the load-carrying capacity was reduced to 15 pounds, a value indicating no significant lubricating properties. It is to be noted that although quebracho was used in this test to simulate the conventional caustic soda-quebracho treatment in the field, the use of quebracho alone without caustic soda will not result in a reduction of the load-carrying capacities of the muds of the invention.

It is significant to note in the above table that, in every instance where there is set forth a composition in accordance with the invention, the load-carrying capacity is always at least 35 pounds. This indicates that the muds of my invention have desirable lubricating properties. The examples also show the variation in the amount of asphalt with its sulfur content. When employing manjak, a high sulfur content asphalt, smaller amounts of asphalt, say from 10 to 20 percent by weight of the oil phase, are utilized. When employing the Kuwait reduced crude containing smaller amounts of sulfur, larger amounts of asphalt are utilized, say from about 40 to 75 percent by weight of the oil phase. Example 10 shows that when using insufficient asphalt to provide at least about one percent of sulfur in the oil phase, the resulting drilling mud has no significant lubricating properties.

It is obvious from the foregoing detailed description of the invention that I have provided superior oil-in-water emulsion drilling muds of improved lubricating properties, which prolong the useful life of drill bits by substantially retarding failure of the bearing thereof. It is therefore now possible to reduce the number of round trips required for replacing drill bits, to reduce the time lost in making bit changes, and thereby to achieve substantial economies in well drilling operations. Furthermore, since fewer bits are required to drill a well, there will be less wear and tear on the drilling rig, and a relatively small, but nevertheless significant savings in the cost of bits. Also, more time will be made available to the drilling crew for performing other essential tasks. When employing the drilling muds of my invention, the limiting factor of bit life is not the bearings, as in the past, but the cutting teeth of the bit. The use of the drilling muds of the invention therefore confers the additional advantage of imparting a safety factor in drilling operations because a bearing failure may not be expected until after the teeth of the bit have been substantially worn out. Since bit changes will be accomplished because of tooth wear prior to the bearings approaching a dangerous condition of wear, the likelihood of cone-fishing jogs is substantially reduced.

It is a further important advantage of the oil-in-water emulsion drilling muds of this invention that the oil phase thereof is capable of preferentially wetting metal surfaces. This ability of the oil phase preferentially to wet metals results in the formation of a continuous film of oil phase on the surfaces of the drill bit and the bearings thereof to the virtual exclusion of water. Accordingly, only relatively small amounts of oil phase, such as are customarily used in oil-in-water emulsion drilling muds, are necessary to obtain the desired lubrication of the bearings of a drill bit in accordance with the invention. When it is considered that the main lubricating function desired of the drilling mud is directed to the small area of metal surface which constitutes the bearings of a drill bit, it will be appreciated that substan-

tial economies are achieved by using the oil-in-water emulsion muds of the invention, particularly since the additives conferring the desired lubricating properties need be based only on the oil phase and not on the entire mud.

As will be apparent to those skilled in the art, conventional modifying agents can be added to my drilling muds without departing from the spirit of the invention, provided that the muds remain substantially free of alkali metal hydroxide. Thus, there can be added the usual weighting agents, viscosity modifiers, agents for reducing fluid loss, etc.

Furthermore, I can add to the muds of this invention containing an asphalt having chemically combined sulfur, as set forth herein, other materials which have a contributory effect on the lubricating properties of the resulting muds. For example, as described and claimed in my copending application Serial No. 465,417, filed on even date herewith, water-insoluble, oil-soluble sulfurized organic compounds are effective in conferring improved lubricating properties on oil-in-water emulsion drilling muds. Also, as described and claimed in my copending application Serial No. 465,419, filed on even date herewith, certain water-insoluble, preferentially oil-wettable inorganic sulfides are effective in conferring lubricating properties on oil-in-water emulsion drilling muds.

I can add to or substitute for part of the asphaltic materials having chemically combined sulfur of the present invention the sulfurized organic compounds or the inorganic sulfides of the above copending applications, or mixtures of these materials, as may be dictated by considerations of cost and availability.

Resort may be had to such other modifications and variations as fall within the spirit of the invention and the scope of the appended claims.

I claim:

1. A drilling mud of enhanced lubricating properties comprising an oil-in-water emulsion containing clay solids, an asphalt in the oil phase, said asphalt having chemically combined sulfur and being present in an amount sufficient to provide at least about one percent of sulfur by weight of the oil phase, said mud containing no amount of alkali metal hydroxide sufficient to destroy the enhanced lubricating properties of the mud.

2. The drilling mud of claim 1, wherein said asphalt has a sulfur content of at least about 1.5 percent and is present in an amount not greater than 75 percent by weight of the oil phase.

3. The drilling mud of claim 2, wherein said asphalt is an asphaltite.

4. The drilling mud of claim 2, wherein said asphalt is a natural asphalt.

5. The drilling mud of claim 2, wherein said asphalt is an asphalt-containing petroleum residue.

6. The drilling mud of claim 2, wherein said asphalt is a reduced crude and is cut back with a gas oil in proportions of reduced crude to gas oil ranging from 1:1 to 3:1.

7. The drilling mud of claim 3, wherein the oil phase of said mud is a residual fuel oil and said asphalt is present in said residual fuel oil.

8. A drilling mud of enhanced lubricating properties comprising an oil-in-water emulsion containing clay solids, an asphalt in the oil phase, said asphalt having chemically combined sulfur and being present in an amount sufficient to provide at least about one percent of sulfur by weight of the oil phase, and an emulsifying agent selected from the group consisting of preferentially oil-soluble alkylarylsulfonic acids and metal salts thereof, the sodium soaps of tall oil, and the higher fatty acid esters of the anhydroalkitols, the amount of emulsifying agent being sufficient to reduce the surface tension of the filtrate substantially below that of water, said mud containing no amount of alkali metal hydrox-

ide sufficient to destroy the enhanced lubricating properties of the mud.

9. The drilling mud of claim 8, wherein the emulsifying agent comprises the sodium salts of mahogany acids.

10. The drilling mud of claim 8, wherein the emulsifying agent comprises sorbitan monooleate.

11. The drilling mud of claim 8, wherein the emulsifying agent comprises the sodium soaps of tall oil.

12. The drilling mud of claim 8, wherein the emulsifying agent comprises mahogany acids.

13. A drilling mud of enhanced lubricating properties comprising an emulsion of a distillate petroleum oil in water, said emulsion containing clay solids, and also containing an asphalt in the oil phase having at least about 1.5 percent by weight of chemically combined sulfur, said asphalt being present in an amount sufficient to provide at least about one percent of sulfur by weight of the oil phase, said mud containing no amount of alkali metal hydroxide sufficient to destroy the enhanced lubricating properties of the mud.

14. The drilling mud of claim 13, wherein the asphalt is a reduced crude and is employed in an amount of from about 40 to 75 percent by weight of the oil phase.

15. The drilling mud of claim 13, wherein there is present an emulsifying agent selected from the group consisting of preferentially oil-soluble alkylarylsulfonic acids and metal salts thereof, the sodium soaps of tall oil, and the higher fatty acid esters of the anhydroalkitols, the amount of emulsifying agent being sufficient to reduce the surface tension of the filtrate substantially below that of water.

16. A drilling mud of enhanced lubricating properties comprising an oil-in-water emulsion containing clay solids and from about 1 to 4 pounds per barrel of mud of an emulsifying agent selected from the group consisting of preferentially oil-soluble alkylarylsulfonic acids and metal salts thereof, the sodium soaps of tall oil, and the higher fatty acid esters of the anhydroalkitols, the oil phase of said emulsion constituting from 5 to 25 percent by volume of said drilling mud and comprising a uniform blend of from about 40 to 75 percent of a sulfur-containing reduced crude oil by weight and a petroleum distillate fraction, the sulfur content of said reduced crude being sufficient to provide at least about one percent of sulfur by weight of the oil phase, said mud containing no amount of alkali metal hydroxide sufficient to destroy the enhanced lubricating properties of the mud.

17. The drilling mud of claim 16, wherein the reduced crude is a Kuwait reduced crude from the Burgan field and has a sulfur content content of about 5 percent.

18. A uniform blend of oily materials, useful in the

oil phase of an oil-in-water emulsion drilling mud of enhanced lubricating properties, comprising an oil, an asphalt containing at least about 1.5 percent of sulfur by weight, and an emulsifying agent, said blend containing no amount of alkali metal hydroxide sufficient to destroy the enhanced lubricating properties of the mud.

19. A process for enhancing the lubricating properties of a drilling fluid during the drilling of a well, drilling of said well having been begun with a water-base drilling mud, which comprises adding to said water-base drilling mud in the drilling fluid system of said well, an oil, an emulsifying agent, and an asphalt having chemically combined sulfur in amounts effective to convert said water-base drilling mud to an oil-in-water emulsion drilling mud containing at least about one percent of sulfur by weight of the oil phase, said mud containing no amount of alkali metal hydroxide sufficient to destroy the enhanced lubricating properties of the mud, circulating the resulting mixture through said drilling mud system, and continuing drilling of the well.

20. The process of claim 19, wherein the emulsifying agent is selected from the group consisting of preferentially oil-soluble alkylarylsulfonic acids and metal salts thereof, the sodium soaps of tall oil, and the higher fatty acid esters of the anhydroalkitols.

21. A process of drilling a well with a rotary bit which comprises forming a borehole with said bit while circulating a drilling mud of enhanced lubricating properties through said borehole, said drilling mud comprising an oil-in-water emulsion containing clay solids, an asphalt in the oil phase, said asphalt having chemically combined sulfur and being present in an amount sufficient to provide at least about one percent of sulfur by weight of the oil phase, said mud containing no amount of alkali metal hydroxide sufficient to destroy the enhanced lubricating properties of the mud.

#### References Cited in the file of this patent

#### UNITED STATES PATENTS

40 2,423,144 Gregg \_\_\_\_\_ July 1, 1947  
2,689,219 Menaul \_\_\_\_\_ Sept. 14, 1954

#### FOREIGN PATENTS

45 476,310 Canada \_\_\_\_\_ Aug. 21, 1951

#### OTHER REFERENCES

50 Davey: The Mechanism of Action of Extreme Pressure Lubricants, article in Scientific Lubrication, Sept. 1949, pages 7, 8, 11 and 14.

Rogers: Composition and Properties of Oil Well Drilling Fluids, Revised Edition, pub. 1953 by Gulf Pub. Co. of Houston, Texas, pages 511, 513, and 514.